

## UNITED STATES PATENT OFFICE

2,412,956

LUBRICANT CONTAINING ALKYL  
PIPERIDINE SALTS

George E. Barker, Pittsburgh, Pa., assignor to  
Elgin National Watch Company, Elgin, Ill., a  
corporation of Illinois

No Drawing. Application August 3, 1944,  
Serial No. 547,979

8 Claims. (Cl. 252—34.7)

1

It is known that when relatively moving surfaces are supplied with an interposed lubricant, the coefficient of friction is normally reduced to a value which is essentially determined by the characteristics of the lubricating agent, the smoothness or polish of the surface, and the materials by which the surfaces are presented. Under conditions of boundary lubrication with given surfaces, the lubricating agent may be selected for certain other desired chemical and physical factors and thus may have an undesirably high coefficient of friction.

It has now been found that a relatively low coefficient of friction may be conferred upon many lubricating agents, without harm to other desired chemical and physical attributes, by adding as an "oiliness" agent a small proportion of a N-alkyl piperidine salt of a fatty acid. Such mixtures are as non-corrosive as the basic lubricating agent and are stable and homogeneous under all normal operative conditions for the selected basic lubricating agent, which for some of the materials can cover the range of temperatures between minus 60 degrees and plus 150 degrees F. The additive also has the effect of improving the rust inhibition, thereby reducing or eliminating the quantity of inhibitor which preferably is added e. g. to ester type or ester containing lubricants.

The basic lubricating agent employed in accordance with this invention is a fluid organic composition containing aliphatic groups. This includes the lubricating oils of mineral origin, commonly known as paraffin and naphthalene base oils, together with lubricating oils of animal, vegetable and marine origin such as neat's foot, porpoise, sperm, castor, etc., oils, and the lubricants set out in my copending application Ser. No. 372,136, now United States Patent No. 2,355,616.

The oiliness agents are in general waxy solids or viscous liquids, by themselves, which are essentially insoluble in water but soluble in the fat solvents and in organic lubricants. They may be prepared by thoroughly mixing, in liquid form, equivalent amounts of the fatty acid and the alkyl piperidine.

## EXAMPLE I

A mixture of 6.2 grams (0.02 mole) of cetyl-piperidine and 5.7 grams (0.02 mole) of stearic acid was warmed in an oven (80 degrees C.) until the stearic acid was completely melted and dissolved in the cetyl piperidine. The liquid was thoroughly stirred to insure homogeneity and

reaction, and allowed to cool to a nearly colorless wax-like solid.

## EXAMPLE II

5 An 88.6 gram (0.312 mole) batch of stearic acid was melted in an oven (80 degrees C.). To the melted solid was added 79 grams (0.312 mole) of dodecyl-piperidine, with vigorous stirring. The product on cooling remained a liquid for about 48 hours before crystallizing to a slightly yellow 10 waxy solid.

## EXAMPLE III

A mixture of 5.96 grams (0.02 mole) of ricinoleic acid and 5.06 grams (0.02 mole) of dodecyl-piperidine was thoroughly agitated and allowed to stand for twenty-four hours. The product was a yellow viscous oil.

The fatty acid should have at least 5 carbon atoms (e. g. valeric acid) to avoid possible water 15 solubility or attack which may occur with the salts of acids containing 4 or less carbon atoms, and the upper limit of carbon content is around 30 atoms as the higher members give compounds which have poor solubility in petroleum lubricants at low temperatures. Saturated straight-chain aliphatic acids, together with branch chain acids having methyl, ethyl, etc., groups in the branch or branches, such as 2-ethyl-hexoic acid, 20 unsaturated acids such as erucic, oleic, undecylenic, etc., and hydroxyl-substituted acids such as ricinoleic, can be used, within the prescription of having 5 to 30 carbon atoms.

The alkyl substituting group in the piperidine complex likewise preferably has 5 to 30 carbon atoms, although as low as a methyl group has 35 been found to exhibit the effect of increasing the oiliness though not to the extent of the preferred groups. The group should have at least 5 carbon atoms, connected to the nitrogen atom of the 40 piperidine ring. The term "piperidine" also includes herein compounds in which hydrogen attached to carbon atoms of the ring has been replaced by alkyl groups such as methyl, etc. 2-ethyl-butyl, 2-ethylhexyl and higher membered 45 chains and branches, that is, branched chain groups, can be employed.

In general, it is preferred to have from 11 to 26 carbon atoms in the acid chain, and 11 to 16 carbon atoms in the alkyl chain.

Such oiliness agents are customarily employed 50 in proportions of 0.05 to 1.0 percent by weight of the lubricant. In general, after a particular quantity has been added, the increase of effect diminishes as more is added. Mixtures of alkyl 55 piperidine salts, each of the type above described,

may be employed. In preferred preparations, the salts are present as groups of isomers, whereby low melting points are assumed.

Comparative effects of the presence of the oiliness agent and specific examples of composition are indicated in the following table:

TABLE  
Coefficients of friction of steel on sapphire,  
lubricated

| Lubricant                                                                        | Coeff. of<br>frict. |
|----------------------------------------------------------------------------------|---------------------|
| Pennsylvania oil, Alchlor treated 21.7 c. s. at 100° F.                          | 0.112               |
| Same oil+0.2 per cent dodecylpiperidine stearate                                 | 0.094               |
| Same oil+0.2 per cent dodecylpiperidine laurate                                  | 0.101               |
| Same oil+0.2 per cent dodecylpiperidine erucate                                  | 0.096               |
| Same oil+0.2 per cent dodecylpiperidine cerotate                                 | 0.093               |
| Same oil+0.2 per cent dodecylpiperidine ricinoleate                              | 0.099               |
| B-amylthioethyl B'-benzylthioethyl ether                                         | 0.124               |
| B-amylthioethyl B'-benzylthioethyl ether+0.5 per cent dodecylpiperidine stearate | 0.0675              |
| Benzyl phenylundecanoate                                                         | 0.109               |
| Benzyl phenylundecanoate+0.2 per cent dodecylpiperidine stearate                 | 0.097               |
| Phenoxyphenyl cetane                                                             | 0.107               |
| Phenoxyphenyl cetane+0.5 percent dodecylpiperidine stearate                      | 0.098               |
| n-Amyl phenylundecanoate                                                         | 0.114               |
| n-Amyl phenylundecanoate+0.5 per cent dodecylpiperidine ricinoleate              | 0.104               |
| 40 parts diethylene glycol dicaproate                                            | 0.123               |
| 60 parts benzyl phenylundecanoate                                                | 0.0976              |
| 0.1 part tert-butyl catechol                                                     |                     |
| 40 parts diethylene glycol dicaproate                                            |                     |
| 60 parts benzyl phenylundecanoate                                                |                     |
| 0.1 part tert-butyl catechol                                                     |                     |
| 0.5 part cetylpiridine stearate                                                  |                     |

From this it will be noted that the coefficient of these lubricants, already low, can be reduced 10 percent or more by the action of the oiliness agent.

The alkyl piperidines may be prepared in various ways. For example, such preparations may proceed:

A. *Dodecylpiperidine*.—44 grams (0.52 mole) of piperidine were mixed with 45 cc. of water in a 500 cc. round bottomed flask fitted with an efficient reflux condenser and a dropping funnel. 140 grams (0.56 mole) of normal dodecyl bromide (prepared in accordance with Organic Synthesis, Collective Volume I, page 29 (1941), John Wiley & Sons Company, New York) were added to the solution in the flask, and the resulting two-phase mixture was heated to refluxing. Then, while the contents of the flask were kept at reflux, there was slowly added through the dropping funnel a solution of potassium hydroxide in 51 cc. of water. Refluxing was continued for three hours after completion of the addition of the potassium hydroxide solution. When the mixture had cooled, the aqueous layer was separated and discarded, and the oil was distilled over solid potassium hydroxide (10 g.). The material boiling between 135 degrees C. and 160 degrees C. at a pressure of approximately 1 mm. of mercury was collected and was redistilled. During the redistillation, the fraction boiling between 120 degrees C. and 140 degrees C. under a pressure of about 1 mm. of mercury was collected as product. The higher boiling point in the initial distillation was presumably caused by superheating due to distilling the dodecylpiperidine out of the

fused potassium hydroxide in the still. The yield of dodecylpiperidine was 79 percent of the theoretical (104 g.).

B. *Cetylpiridine*.—The procedure is exactly as above for dodecylpiperidine, except that cetyl chloride, in corresponding molecular proportion, was substituted for the dodecyl bromide. The product, cetylpiridine, distilled between 160 degrees C. and 175 degrees C. under a pressure of approximately 1 mm. of mercury. It showed a melting point of 19-20 degrees C.

It will be understood that the invention is not limited to the illustrated practices, but may be practiced in many ways within the scope of the appended claims.

I claim:

1. A lubricant consisting of an organic lubricant liquid having dissolved therein from 0.05 to 1.0 percent of an alkyl-piperidine salt of a fatty acid, the alkyl group having from 5 to 30 carbon atoms and the acid group having from 5 to 30 carbon atoms.

2. A lubricant consisting of a hydrocarbon oil lubricant having dissolved therein from 0.05 to 1.0 percent of dodecylpiperidine stearate.

3. A lubricant comprising in major part an ester of an aryl-substituted carbon-chain acid having dissolved therein from 0.05 to 1.0 percent of an alkyl-piperidine salt of a fatty acid, said acid group having from 5 to 30 carbon atoms, the said alkyl group having from 12 to 16 chain carbon atoms.

4. A lubricant consisting essentially of an organic lubricant liquid having dissolved therein from 0.05 to 1.0 percent of an alkyl-piperidine salt of ricinoleic acid, the said alkyl group having from 12 to 16 chain carbon atoms.

5. A lubricant consisting essentially of an organic lubricant liquid having dissolved therein from 0.05 to 1.0 percent of an alkyl-piperidine stearate.

6. A lubricant consisting of an organic lubricant liquid consisting at least in major part of an aralkyl compound having at least five carbon atoms in an aliphatic chain, together with about 0.5 part of an alkyl-piperidine salt in which the piperidine alkyl group contains five to thirty carbon atoms in chain connected to the nitrogen atom of the piperidine ring and in which the acid group of the salt is an aliphatic acid having five to thirty carbon atoms.

7. A lubricant consisting of an organic lubricant liquid consisting at least in major part of an aralkyl compound having at least five carbon atoms in an aliphatic chain, together with about 0.5 part of an alkyl-piperidine salt in which the piperidine alkyl group contains from 11 to 16 carbon atoms in chain connected to the nitrogen atom of the piperidine ring and in which the acid group of the salt is an aliphatic acid having 11 to 26 carbon atoms.

8. A lubricant consisting essentially of a mixture of substantially 40 parts of diethylene glycol dicaproate and 60 parts of benzyl phenylundecanoate, together with about 0.5 parts of cetyl-piperidine stearate.

GEORGE E. BARKER.